

## UNITED STATES PATENT OFFICE

2,330,775

## NOVEL DYEING EFFECTS

Louis H. Bock, Huntingdon Valley, and Alva L. Houk, Philadelphia, Pa., assignors to Röhm & Haas Company, Philadelphia, Pa.

No Drawing. Application March 12, 1941,  
Serial No. 382,940

8 Claims. (Cl. 8—120)

This invention relates to a method for producing novel coloring effects in textile fabrics containing cellulosic fibers or regenerated cellulosic fibers. In particular, this invention deals with creating effects in the dyeing of fabrics containing cotton, linen, ramie, other cellulosic fibers or regenerated cellulosic fibers by altering the capacity for dyes of at least a part of said fibers by reaction with a quaternary ammonium compound having as an N-substituent at least one 10 oxymethyl group.

It has previously been proposed to render cellulose fibers indifferent to substantive cotton colors by esterifying such fibers with an agent such as toluene sulfonyl chloride, benzoyl chloride, or acetic anhydride. In general, such prior processes have required complicated procedures, excessively long periods of treatment, or techniques which are scarcely practical in the average textile mill. As a result of such processes, fabrics have been unduly tendered at times and the fabrics so treated have been seriously changed in their physical appearance and properties. Such disadvantages are avoided by the method herein described for altering the susceptibility of cellulosic fibers to dyestuffs.

In accordance with the present invention decorative and novel effects are obtained in textile fabrics containing cellulosic fibers by treating at least part of the cellulosic material making up the fabric with a quaternary ammonium compound having at least one oxymethyl group having a substituent of 7 to 14 carbon atoms, heating the treated cellulosic material to cause a reaction between it and the said salt, and subsequently applying a dye to the treated and heated material. When the dye applied is one which is normally substantive to cotton, the cellulosic material exhibits a reserve effect and is but slightly colored. On the other hand, the treated and heated material accepts dyes of the acetate type.

If a cotton fabric is woven in part with untreated, normal yarns and in part with yarns which have been treated and heated as described, patterns are obtained when the cloth is dyed with a single dye. The treated and untreated fibers or yarns differ in color, intensity of color or shade. Novel effects may also be obtained by printing cellulosic fabrics with pastes containing a quaternary ammonium compound having an oxymethyl group with a substituent of 7 to 14 carbon atoms, heating the printed fabric to cause a reaction between fabric and said compound, and then dyeing the fabric to give patterns. Novel effects are also obtained in cross dyeing.

The quaternary ammonium compounds which are useful in this invention have the general formula



wherein R is an aliphatic, cycloaliphatic, or an aralkyl group having 7 to 14 carbon atoms, X is an anion, and R<sub>1</sub>, R<sub>2</sub>, and R<sub>3</sub> are organic groups selected to satisfy three valences of the nitrogen from at least one member of the class consisting of trivalent unsaturated hydrocarbon chains which jointly with the nitrogen form a heterocycle, divalent saturated aliphatic chains which jointly with the nitrogen form a heterocycle and monovalent cycloaliphatic, araliphatic, and aliphatic groups.

20 Suitable groups for R include n-octyl, iso-octyl,  $\alpha, \alpha, \gamma, \gamma$ -tetramethyl butyl, decyl, undecenyl, dodecyl, hydrocarbon groups from commercial cuts of alcohols having 7 to 14 carbon atoms, obtained, for example from hydrogenated fatty 25 glycerides, or from the alcohols of the methanol-catalytic synthesis, methyl cyclohexyl, cyclohexylcyclohexyl, butylcyclohexyl, benzyl, methyl benzyl, butyl benzyl, etc. Typical groups occurring as X are the chloride, bromide, iodide, formate, acetate, sulfate, ethyl sulfate, hydroxide, etc. groups. While the halide salts are most readily prepared, it is possible through the hydroxide to form salts with any acid, whether strong or weak, organic or inorganic. The nature of R<sub>1</sub>, R<sub>2</sub>, 30 and R<sub>3</sub> may be widely varied. When the three groups are taken as a trivalent radical, they constitute an unsaturated hydrocarbon chain as is found in pyridine, quinoline, picoline, or the like. When two of the groups together represent a divalent saturated aliphatic radical, this radical 35 forms with the nitrogen a heterocycle such as occurs in piperidine, morpholine, pyrrolidine, or the like. With such a divalent group there is, of course, required a monovalent group to satisfy the 40 remaining valences of the nitrogen. When R<sub>1</sub>, R<sub>2</sub>, or R<sub>3</sub> represent monovalent groups, they may 45 represent aliphatic, cycloaliphatic, or araliphatic groups. Typical aliphatic groups include not only saturated and unsaturated open chain hydrocarbons but also aliphatic groups carrying such functional groups as hydroxyl, halogen, amide, nitrile, ester, ether, aldehyde, ketone, amino, etc. Typical araliphatic groups include benzyl, methylbenzyl, phenoxyethyl, methyl phenoxyethoxyethyl, ethoxyphenoxyethyl, etc., while typical of the 50 55

cycloaliphatic groups are the cyclohexyl and methyl cyclohexyl radicals.

Some of the types of compounds which have been found useful in this application of quaternary ammonium salts are as follows:



Although quaternary ammonium compounds having oxymethyl groups with substituents of 7 to 14 carbon atoms are generally suitable for the purposes of this invention, those compounds having such substituents with 10 to 12 carbon atoms are the most effective.

In using the quaternary ammonium compounds having an oxymethyl group to alter the capacity of cellulosic materials for dyes, it is necessary to use fairly concentrated solutions thereof, a concentration of about 10% or more being usually required. The range of 10% to 25% is preferred. The quaternary compound may be dissolved in water, an organic solvent such as ethyl alcohol or acetone, or in a mixture of solvent and water. The solution may be applied to fiber, yarn, or fabric by spraying, spreading, immersing, printing, or other suitable mode of application. Excess solution may be removed by squeezing, centrifuging, vacuum extracting, or equivalent procedure. The impregnated material is dried and baked at a temperature between about 100° C. and about 160° C. The lower temperature is determined by that at which the desired reaction is effected. The permissible upper temperature must be below that at which scorching of fabric would occur with regard to the particular cellulosic material or fabric being treated and the time required to effect the reaction. Following the reaction it is often desirable to wash the treated material to remove unreacted quaternary compound and reaction products remaining from combining the long chain oxymethyl group with the cellulose. The treated material is subsequently subjected to the action of a dye bath according to any of the usual procedures. If the treated cellulosic materials are in the form of fibers or yarns, they are usually, but not necessarily, made into cloth before the dyeing step. Where printing is involved or in cases where cellulosic yarns are woven or knitted with other types of fibers, the treating may, of course, be done with the fabric itself.

The resulting dyed fabric exhibits differential dyeing effects, since the treated portions or parts have a different affinity for dyes than untreated portions or parts. Against such dyes as vat dyes, sulfur dyes, and direct cotton dyes, treated cellulosic material exhibits a reserve effect, while

against such dyes as direct acetate dyes, an increased affinity is exhibited.

The following examples further describe the invention and give illustrative details.

#### EXAMPLE 1

A skein of cotton yarn was immersed in a 10% aqueous solution of dodecyloxymethyl butyloxymethyl dimethyl ammonium chloride, dried at room temperature and heated in an oven at 130° C. for 30 minutes, rinsed in water, and dyed for 30 minutes at 100° C., in a bath containing 1% Diazine Black OB. Diazine Black OB is listed in the Yearbook of the American Association of Textile Chemists and Colorists as belonging to Foreign Prototype 147. The skein so treated was only lightly colored. A second skein of cotton yarn which was not so immersed in the aqueous solution but which was subjected to the same dyeing bath for the same period of time and at the same temperature was dyed a deep black.

Another skein of cotton yarn was immersed in a 20% aqueous solution of the same quaternary ammonium compound and treated as above. This skein showed even greater resistance to dyeing with Diazine Black OB under the same conditions of time, temperature and concentration.

#### EXAMPLE 2

A piece of cotton sheeting was immersed in a 20% aqueous solution of octyloxymethyl benzyl-oxyethyl dimethyl ammonium chloride, thereafter dried for ten minutes in an oven at 130° C., and then heated for ten minutes in an oven at 150° C. After the heat treatment the cloth was washed with a soap solution, rinsed in water several times, and dyed for 30 minutes at 100° C. in a bath containing 1% Diazine Black OB. The resulting cloth was a light, pearl gray.

A piece of cotton sheeting, not treated with the quaternary ammonium salt but dyed in the same bath for the same length of time and at the same temperature, became a rich black in color.

In the same way pieces of the original sheeting and pieces of the sheeting impregnated and heated with octyloxymethyl benzyl-oxyethyl dimethyl ammonium chloride were dyed with Benzofast Scarlet 4BSA (Color Index No. 327) and with Pontamine Sky-blue 6B (Color Index No. 518). The original fabric, untreated with a quaternary compound, became deep red and royal blue in the two dye baths respectively, while the treated pieces were only lightly tinted.

#### EXAMPLE 3

Kier-boiled and bleached percale was padded through a 20% aqueous solution of dodecyloxymethyl ethoxyethyl dimethyl ammonium chloride, dried in a frame, and heated in a drier at 130° C. for about 20 minutes, and thereafter washed in soap solution and rinsed. Pieces of this fabric were then treated in baths of dyes of different types and a piece of the original percale was also entered in each dye bath for purposes of comparison.

(a) A bath was prepared from 2 parts of tetrabromoindigo (Color Index No. 1184), 2.5 parts of sodium hydrosulfite, 10 parts of a 20% aqueous sodium hydroxide solution, and 100 parts of water by heating the mixture at 70° C. until reduction was complete, and then diluting with 200 parts of boiled water. Pieces of both treated and original fabric were padded through this solution, thereafter treated in an oxidizing bath, and dried. The original untreated fabric was a

full blue, while the treated fabric acquired only a light shade.

(b) Pieces of original percale and treated percale were dyed for one hour in a bath at 70° C., containing 5 parts of SRA Orange III, an acetate dye, 0.5 part of soap, and 200 parts of water. The original fabric held only a trace of dye while the treated fabric acquired a deep, full color.

10 A piece of fabric composed of cellulose acetate was also dyed in the SRA Orange III bath. It became bright red.

15 (c) Other pieces of original and treated fabrics were steeped for one-half hour at 100° C., in a bath composed of 5 parts of Calcogene Dark Brown N, 5 parts of sodium sulfide and 200 parts of water. The treated piece retained very little of the dye while the control was a black-brown.

#### EXAMPLE 4

20 An all-spun rayon fabric was padded through a warm 15% solution of octyloxymethyl butyloxymethyl morpholinium chloride, dried, heated for 20 minutes in an oven at 150° C., and thereafter laundered in hot soap solution, rinsed, and entered in a bath containing 1% of Diazine Black OB, held between 80° and 100° C. The treated fabric took up very little dye, while a piece of the fabric, subjected to the same dye bath under the same conditions but which had not been preliminarily treated, became black.

#### EXAMPLE 5

30 (a) A piece of spun rayon fabric was impregnated with a 20% aqueous solution of capryloxy-35 methyl dimethyl benzyl ammonium hydroxide, dried at room temperature, heated in an oven at 130° C. for one-half hour, and washed. It was then entered into a dye bath containing Benzofast Scarlet 4BSA and treated for one-half hour at 100° C. Practically no dye was taken up by the fabric, whereas a piece of the original fabric in the dye bath became a brilliant red.

40 (b) A rayon taffeta was padded through a solution containing 20% of capryloxyethyl dimethyl benzyl ammonium hydroxide, dried at low temperature, heated in oven at 140° C. for one-half hour, and washed. It was then treated in a bath containing SRA Orange III, a celanese dye, and treated for an hour at 70° C. A deep orange-brown color was imparted to the treated fabric whereas an untreated piece of the original fabric retained very little of the dye.

45 (c) A piece of spun viscose rayon fabric was treated in a 10% aqueous solution of capryloxy-55 methyl dimethyl benzyl ammonium hydroxide, dried at low temperature, heated in an oven at 130° C. for one-half hour, and washed. It was then treated in a bath of SRA Orange III for one hour at 70° C. An orange-brown color was 60 imparted to the fabric and the color was well retained.

The alteration of the dyeing properties of regenerated cellulose is most marked when quaternary ammonium hydroxides are used or the treating solution contains both hydroxide and salt forms. On the other hand, cotton is most effectively treated in this process with the salts.

65 By generally similar procedures the effects were demonstrated of treating different cellulosic materials with a variety of dyes. This work is summarized in the following table, in the columns of which are shown the nature of quaternary compound used, its concentration; the fabric to which it was applied, the treatment of the impregnated fabric, the dye applied to the

treated fabric, and the resulting color. In all cases it will be noted the treated fabric responded differently from the original fabric.

It should be noted that the differential dyeing effects are due to an actual chemical modification of part of the cellulosic material, the altera-

TABLE I  
*Summary of treating fabrics with various salts and dyeing*

| Compound                                                                     | Concn.   | Fabric | Heated          | Dye used                | Result             |
|------------------------------------------------------------------------------|----------|--------|-----------------|-------------------------|--------------------|
| Dodecyloxymethyl butoxymethyl dimethyl ammonium chloride.                    | Per cent |        |                 |                         |                    |
| Do.                                                                          | 20       | Cotton | 1/2 hr. 130° C. | Benzo-fast Scarlet 4BSA | V. lt. pink.       |
| Do.                                                                          | 20       | Linen  | do              | do                      | Do.                |
| Do.                                                                          | 20       | Cotton | 8 min. 150° C.  | do                      | Pale pink.         |
| Do.                                                                          | 20       | do     | 1/2 hr. 110° C. | Pontamine Diazo Black   | Lt. blue-gray.     |
| Do.                                                                          | 20       | do     | 1/2 hr. 130° C. | SRA Orange III          | Deep orange-brown. |
| Do.                                                                          | 20       | do     | do              | Pontamine Skyblue 6B    | Pale blue.         |
| Do.                                                                          | 20       | do     | do              | CalcoGene Dark Brown N  | Light brown.       |
| Do.                                                                          | 20       | do     | 1/2 hr. 140° C. | Tetrabromo-indigo       | Light blue.        |
| Do.                                                                          | 10       | do     | 1/2 hr. 130° C. | Pontamine Diazo Black   | Medium gray.       |
| Dodecyloxymethyl benzyloxymethyl dimethyl ammonium chloride.                 | 20       | do     | do              | do                      | Pale gray.         |
| Dodecyloxymethyl methallyloxymethyl dimethyl ammonium chloride.              | 20       | do     | do              | do                      | Light gray.        |
| Dodecyloxymethyl butoxymethyl piperidinium chloride.                         | 20       | do     | do              | do                      | Medium gray.       |
| Diisobutylphenoxyethoxyethyl octyloxymethyl dimethyl ammonium chloride.      | 20       | do     | do              | do                      | V. pale pink.      |
| Dodecyloxymethyl pyridinium chloride.                                        | 20       | do     | do              | do                      | Do.                |
| Do.                                                                          | 20       | Linen  | do              | do                      | Med. orange-brown. |
| Do.                                                                          | 20       | Cotton | do              | Pontamine Diazo Black   | V. pale gray.      |
| Benzylloxymethyl dimethyl benzyl ammonium chloride.                          | 20       | do     | do              | SRA Orange III          | Med. orange-brown. |
| Dodecyloxymethyl dimethyl benzyl ammonium chloride.                          | 20       | do     | do              | do                      | Dark brown.        |
| Do.                                                                          | 20       | do     | do              | Benzo-fast Scarlet 4BSA | Pale pink.         |
| Dodecyloxymethyl triethyl ammonium chloride.                                 | 20       | do     | do              | Pontamine Diazo Black   | Pale gray.         |
| Dodecyloxymethyl dibenzyl methyl ammonium chloride.                          | 20       | do     | do              | do                      | Do.                |
| Tetradecyloxymethyl trimethyl ammonium chloride.                             | 20       | do     | do              | do                      | Light gray.        |
| 2-ethylhexyloxymethyl diethyl hydroxyethyl ammonium chloride.                | 20       | do     | do              | do                      | Pale gray.         |
| Dodecyloxymethyl 2-hydroxypropyl dimethyl ammonium chloride.                 | 20       | do     | do              | do                      | Do.                |
| Dodecyloxymethyl dimethyl cyclohexyl ammonium chloride.                      | 20       | do     | do              | do                      | Do.                |
| Dodecyloxymethyl-3-dimethylamino-2-hydroxypropyl dimethyl ammonium chloride. | 20       | do     | do              | do                      | Do.                |
| Dodecyloxymethyl 2-hydroxyethyl morpholinium chloride.                       | 20       | do     | do              | do                      | Do.                |
| Dodecyloxymethyl 2-formylpropyl dimethyl ammonium chloride.                  | 20       | do     | do              | do                      | Med. lt. gray.     |
| Dodecyloxymethyl 2-carbomethoxypropyl dimethyl ammonium chloride.            | 20       | do     | do              | do                      | Pale gray.         |
| Dodecyloxymethyl 2-hydroxyoctyl dimethyl ammonium chloride.                  | 20       | do     | do              | do                      | Med. pale gray.    |
| Dodecyloxymethyl 3-phenylpropyl-3-dimethyl ammonium chloride.                | 20       | do     | do              | do                      | Pale gray.         |

#### EXAMPLE 6

A solution containing about 12% of dodecyloxymethyl pyridinium chloride and 1% of sodium acetate was rubbed through a silk stencil placed over a piece of percale, the stencil permitting transfer of the solution to the percale in local areas. The cloth was then heated for one-half hour at 130° C., washed in soap and water, and placed in a 1% solution of Pontamine Sky-blue 6B for one-half hour at 95-100° C. A design was thus developed in the percale, the treated areas being but lightly tinted while the untreated areas were a deep blue.

For effecting a change in the dyeing properties of cellulose and regenerated cellulose a solution containing about 10% to about 25% of an oxymethyl quaternary ammonium compound is generally required for impregnation and reaction with the cellulosic fibers. The treated fibers may be used along with other fibers to give novel effects in dyeing. The effects may be obtained by combining the treated and altered fibers with untreated fibers of the same origin or with fibers of a different type such as silk, wool, cellulose acetate, etc. Yarns may be treated, woven into a fabric in a pattern and the fabric dyed. Fibers within local areas of a fabric may be altered by printing methods and designs developed on subsequent heating and dyeing. Decorative effects are also obtained by cross dyeing.

tion involving primarily the surface. The operation of the oxymethyl quaternary compounds in the manner here described is different than that with the usual quaternary salts which have been added to dye baths or used in after-treatments to fix certain dyes on various fibers. In these cases the quaternary salts form complexes with the dyes.

In the application of the oxymethyl quaternary ammonium compounds to alter the susceptibility of cellulosic materials to dyes, there may be used in the impregnating solutions salts of weak acids and strong bases, such as sodium acetate, sodium phosphate or the like, or salts of strong acids and weak bases, such as ammonium chloride. These salts may serve as buffers or as catalysts, but are not essential for the successful performance of the process. There may also be added to aqueous solutions an organic solvent to improve solubility and to decrease the viscosity of the solutions.

The nature of the process is such that it may be practised with standard textile equipment without damage thereto and without harm to the fabrics. Results are highly satisfactory and are uniformly and reproducibly obtained.

We claim:

1. A method of producing novel coloring effects in a textile fabric containing fibers selected from the class consisting of cellulose and regenerated cellulose fibers by altering the capacity for dyes

of at least part of said fibers by increasing affinity thereof for acetate dyes and decreasing affinity thereof for direct dyes, which comprises impregnating at least part of said fibers with a solution containing about 10% to about 25% of a compound of the formula



wherein R is a group which contains 7 to 14 carbon atoms and is selected from a member of the group consisting of aliphatic and cycloaliphatic hydrocarbon groups and aralkyl groups, X is an anion, and R<sub>1</sub>, R<sub>2</sub> and R<sub>3</sub> are organic groups selected to satisfy three valences of the nitrogen atom from at least one member of the class consisting of trivalent unsaturated hydrocarbon chains which jointly with the nitrogen form a heterocycle, divalent saturated aliphatic chains which jointly with the nitrogen form a heterocycle, and monovalent cycloaliphatic, araliphatic, and aliphatic groups, heating the impregnated fibers to cause reaction between fibers and compound, and subsequently subjecting the treated fibers to the action of a dye.

2. A method of producing novel coloring effects in a textile fabric containing fibers selected from the class consisting of cellulose and regenerated cellulose by altering the capacity for dyes of at least part of said fibers by increasing affinity thereof for acetate dyes and decreasing affinity thereof for direct dyes, which comprises impregnating at least part of said fibers with a solution containing at least 10% of a compound of



wherein R is a group which contains 7 to 14 carbon atoms and is selected from a member of the group consisting of aliphatic and cycloaliphatic hydrocarbon groups and aralkyl groups, X is an anion, and R<sub>1</sub>, R<sub>2</sub> and R<sub>3</sub> are organic groups selected to satisfy three valences of the nitrogen atom from at least one member of the class consisting of trivalent unsaturated hydrocarbon chains which jointly with the nitrogen form a heterocycle, divalent saturated aliphatic chains which jointly with the nitrogen form a heterocycle, and monovalent cycloaliphatic, araliphatic, and aliphatic groups, heating the impregnated fibers to a temperature between about 100° C. and the temperature at which scorching would occur, and subsequently subjecting fabric containing the treated fibers to the action of a dye.

3. A method of producing novel coloring effects in a textile fabric containing fibers selected from the class consisting of cellulose and regenerated cellulose by altering the capacity for dyes of at least part of said fibers by increasing affinity thereof for acetate dyes and decreasing affinity thereof for direct dyes, which comprises impregnating at least part of said fibers with a solution containing about 10% to about 25% of a compound of the formula



wherein R is selected from a member of the class consisting of aliphatic and cycloaliphatic hydrocarbon groups and aralkyl groups containing 7 to

14 carbon atoms and X is an anion, heating the impregnated fibers to a temperature between about 100° C. and the temperature at which scorching would occur, and subsequently subjecting fabric containing the treated fibers to the action of a dye.

4. A method of producing novel coloring effects in a textile fabric containing fibers selected from the class consisting of cellulose and regenerated cellulose by altering the capacity for dyes of at least part of said fibers by increasing affinity thereof for acetate dyes and decreasing affinity thereof for direct dyes, which comprises impregnating at least part of said fibers with a solution containing about 10% to about 25% of dodecyloxymethyl pyridinium chloride, heating the impregnated fibers to a temperature between about 100° C. and the temperature at which scorching would occur, and subsequently subjecting fabric containing the treated fibers to the action of a dye.

5. A method of producing novel coloring effects in a textile fabric containing fibers selected from the class consisting of cellulose and regenerated cellulose by altering the capacity for dyes of at least part of said fibers by increasing affinity thereof for acetate dyes and decreasing affinity thereof for direct dyes, which comprises impregnating at least part of said fibers with a solution containing about 10% to about 25% of a compound of the formula



wherein R is selected from a member of the class consisting of aliphatic and cycloaliphatic hydrocarbon groups and aralkyl groups containing 7 to 14 carbon atoms, X is an anion, R<sub>1</sub> and R<sub>2</sub> are lower alkyl groups, and R<sub>3</sub> is an aralkyl group, heating the impregnated fibers to a temperature between about 100° C. and the temperature at which scorching would occur, and subsequently subjecting fabric containing the treated fibers to the action of a dye.

6. A method of producing novel coloring effects in a textile fabric containing fibers selected from the class consisting of cellulose and regenerated cellulose by altering the capacity for dyes of at least part of said fibers by increasing affinity thereof for acetate dyes and decreasing affinity thereof for direct dyes, which comprises impregnating at least part of said fibers with a solution containing about 10% to about 25% of dodecyloxymethyl benzyl dimethyl ammonium chloride, heating the impregnated fibers to a temperature between about 100° C. and the temperature at which scorching would occur, and subsequently subjecting fabric containing the treated fibers to the action of a dye.

7. A method of producing novel coloring effects in a textile fabric containing regenerated cellulose fibers by altering the capacity for dyes of at least part of said fibers by increasing affinity thereof for acetate dyes and decreasing affinity thereof for direct dyes, which comprises impregnating at least part of said fibers with a solution containing about 10% to about 25% of a compound of the formula



wherein R is a group which contains 7 to 14 carbon atoms and is selected from a member of the

group consisting of aliphatic and cycloaliphatic hydrocarbon groups and aralkyl groups, and R<sub>1</sub>, R<sub>2</sub>, and R<sub>3</sub> are organic groups selected to satisfy three valences of the nitrogen atom from at least one member of the class consisting of trivalent unsaturated hydrocarbon chains which jointly with the nitrogen form a heterocycle, divalent saturated aliphatic chains which jointly with the nitrogen form a heterocycle, and monovalent cycloaliphatic, araliphatic, and aliphatic groups, heating the impregnated fibers to a temperature between about 100° C. and that at which scorching would occur, and subsequently subjecting fabric containing the treated fibers to the action of a dye.

8. A method of producing novel coloring effects in a textile fabric containing cotton by increasing affinity thereof for acetate dyes and decreasing affinity thereof for direct dyes, which comprises impregnating at least part of the cotton with a 20 solution containing about 10% to about 25% of a compound of the formula



wherein R is a group which contains 7 to 14 carbon atoms and is selected from a member of the class consisting of aliphatic and cycloaliphatic hydrocarbon groups and aralkyl groups, X<sub>1</sub> is a salt-forming anion, and R<sub>1</sub>, R<sub>2</sub>, and R<sub>3</sub> are organic groups selected to satisfy three valences of the nitrogen atom from at least one member of the class consisting of trivalent unsaturated hydrocarbon chains which jointly with the nitrogen form a heterocycle, divalent saturated aliphatic chains which jointly with the nitrogen form a heterocycle, and monovalent cycloaliphatic, araliphatic, and aliphatic groups, heating the impregnated cotton between about 100° C. and about 160° C. to cause reaction between cotton and quaternary ammonium salt, and subsequently subjecting the treated cotton to the action of a dye.

LOUIS H. BOCK.  
ALVA L. HOUK.